

Patented May 18, 1926.

1,584,850

# UNITED STATES PATENT OFFICE.

ALFRED I. CONE, OF NEW YORK, N. Y.

## SAFETY PAPER.

No Drawing.

Application filed May 6, 1925. Serial No. 28,506.

This invention relates to safety papers of the class which are impregnated with or carry various chemical substances intended to produce color reactions when attempts 5 are made to obliterate by chemical means anything written or printed on the surface of such paper.

Numbers of such papers have hitherto been prepared and have generally been confined 10 to providing means for detection when alterations have been attempted with the use of the ordinary devices of treating the written or printed characters on the paper with eradicating fluids, composed of the 15 usual solutions of acids, alkalies, hypochlorite, hyposulphite, etc., but have been open to a number of objections, especially, in that the skilled forger, knowing that he is dealing with a safety paper, can take the pre- 20- cautions of avoiding of counteracting the ordinary color reactions hitherto employed as safety devices.

The present invention, besides providing novel improvements as to the materials to 25 be employed for the purpose of increased efficiency, also provides means for frustrating attempts by subsequent treatments to obliterate the effect of any primary reactions produced when alterations have been 30 attempted, and also means for detection of attempts to remove the chemicals from such safety paper before the application of eradicator fluids, in order to avoid the tell-tale discolorations which would be produced by 35 reactions with such chemicals, when present in the paper. The paper prepared as herein described develops certain color reactions with various chemicals, whereby any attempt to eradicate a character produces unmistakable ocular evidence of an attempt at falsification, etc., and also provides means for 40 showing if an attempt has been made to wash out some of the chemical materials from the paper.

45 The invention consists essentially in combining with the paper certain salts of mercury, preferably insoluble mercurous salts. I have found that insoluble mercurous salts in general are adapted to afford a safety paper of the character described. I prefer to use the insoluble mercurous sulphinate as the salt best adapted for the purpose, and to this end I incorporate the mercurous sulphinate in the pulp before the latter 55 is made into paper.

Such mercurous salt, being insoluble, is obviously not so readily washed away in the process of manufacturing the paper by the usual liquids employed for such purpose. Mercurous sulphinate is also much 60 less liable to discolor the finished paper when exposed to the action of light than when a paper is made with almost all other mercurous salts. A paper thus made with mercurous sulphinate will develop with 65 alkalies a brown or black color; with chlorine or hypochlorites a brownish-red color develops; with thiosulphate (hyposulphite), sulphite, bisulphite, or ammonia, a brownish to black color will develop; if an iodide 70 solution is applied to the paper in an attempt to wash out any contained chemicals, the mercury sulphinate will produce a yellow to black discoloration.

In safety papers of the class described, it 75 is always desirable to provide for a multiplicity of side reactions so as to render it increasingly difficult to make alterations thereon without leaving some evidences of tampering, and the further measures necessary to make such alterations will eventually render a document so unsightly as to defeat the object.

Although the mercurous sulphinate itself affords a high degree of protection, I 85 prefer to add certain other chemicals as an added safeguard. For this purpose I may also use sulphuric acid or a sulphinate and/or benzidine sulphate. When these chemicals are used the benzidine sulphate, 90 which is insoluble in water, as well as in the usual solvents, is incorporated in the pulp in conjunction with the insoluble mercurous salt used, while the sulphinate is applied to the finished paper in the form of a size 95 or impregnating solution.

The impregnating solution referred to is a solution of sulphuric acid or, preferably, a more freely soluble salt thereof.

I have found that sulphuric acid and its 100 soluble salts afford a yellow stain reaction when applied to moistened unbleached or partly bleached ligno-cellulose paper, and I use this reaction as an added protective measure so as to afford means to detect 105 whether any attempt has been made to remove, by washing out the chemicals which have been incorporated. Thus if a check, for instance, has been washed, and the sulphuric constituent thus removed, this can eas- 110

ily be demonstrated by the failure to afford a substantial characteristic yellow stain upon the moistened ligno-cellulose paper when the latter is pressed against the suspected document under investigation.

The benzidine sulphate may also be optionally incorporated in conjunction with the mercurous salt, as an added measure of protection. Benzidine sulphate has been 10 used in the manufacture of safety papers for a number of years, but while it affords a strong reaction with hypochlorite, yet, when used alone, the discoloration thus produced can be readily removed, for instance, 15 by treatment with a sodium hydrosulphite solution.

However, when this well-known benzidine sulphate is incorporated in the pulp in combination with the mercurous salt as 20 above disclosed, then the attempt to remove the benzidine stain will result in the development of a black stain which is practically not removable.

The various color reactions, together with 25 the varied and numerous manipulations that would be required for the removal of the stains developed by them will render the document so unsightly, or impair its appearance to such an extent, as to make it 30 highly unsafe, for instance, to attempt to pass a check or other negotiable instrument made from a paper prepared as herein described and so manipulated.

Any attempt to remove any of the color 35 stains developed as above described will result in either intensifying such color stain, or changing that color stain to another, with the result that the paper becomes still more unsightly and dangerous to pass.

If the paper survives the effort to remove 40 the soluble and insoluble chemicals, the absence of the reaction with the moistened ligno-cellulose paper mentioned above will in itself disclose the fact that the paper has 45 been tampered with.

The sulphaniolate impregnation and the addition of the benzidine sulphate may be dispensed with without disturbing the protection afforded by the insoluble mercurous 50 salt incorporated in the pulp, but manifestly the protection afforded is increased as additional agents are employed, and it is therefore almost always desirable to incorporate those mentioned and even others, according to the degree and character of the 55 protection desired. It is preferable to incorporate about 2% of the insoluble mercurous sulphaniolate in the pulp; of the sulphaniolic acid or a soluble salt of sulphaniolic 60 about 1% should be incorporated in order to afford dependable results; and of the benzidine sulphate about  $\frac{1}{2}\%$  may be incorporated; but the materials can be used in varying quantities according to the in-

tensity of the reactions which it is desired 65 to develop.

Of course excessive quantities of insoluble chemicals used in loading the pulp will impair the quality and the tensile strength of the paper and also increase unnecessarily 70 the cost of the paper.

Obviously also various other chemicals, which will not react with those mentioned herein to impair their efficiency, may be added, optionally, to produce any further 75 special reaction as may be desired. It is not my desire to be limited to any specific combination of materials, as the invention is susceptible of some modifications, as indicated or otherwise apparent, all of which 80 will come within the scope of the invention and without departing from the spirit thereof.

Having thus described my invention, what I claim as new and desire to secure by 85 Letters Patent is:

1. A safety paper containing a mercurous salt.

2. A safety paper containing an insoluble 90 mercurous salt.

3. A safety paper containing mercurous sulphaniolate.

4. A safety paper containing mercurous sulphaniolate and sulphaniolic acid or a soluble 95 salt of sulphaniolic acid.

5. A paper having incorporated therein mercurous sulphaniolate and impregnated with a solution of sulphaniolic acid or a soluble salt of sulphaniolic acid.

6. The process of making a safety paper 100 which consists of incorporating in the pulp mercurous sulphaniolate.

7. The process of making a safety paper which consists of impregnating the paper 105 with mercurous sulphaniolate and sulphaniolic acid or a soluble salt of sulphaniolic acid.

8. The process of making a safety paper by incorporating in the pulp mercurous sulphaniolate and impregnating the paper 110 with sulphaniolic acid or a soluble salt of sulphaniolic acid.

9. A safety paper containing an insoluble mercurous salt and a sulphaniolate.

10. A safety paper containing benzidine sulphate in conjunction with an insoluble 115 mercurous salt.

11. A safety paper containing benzidine sulphate in conjunction with mercurous sulphaniolate.

12. A safety paper containing a substantially insoluble mercurous salt, sulphaniolic acid or a salt thereof, and benzidine sulphate.

13. A safety paper containing mercurous sulphaniolate, sulphaniolic acid or a salt thereof, and benzidine sulphate.

ALFRED I. CONE.